

Feb. 20, 1934.

J. BROADMAN

1,947,516

PROTECTING DOCUMENTS, NEWSPAPERS, AND THE LIKE

Filed Oct. 18, 1932



*Joseph Broadman*  
INVENTOR.

BY *Mock + Bell*  
ATTORNEYS

## UNITED STATES PATENT OFFICE

1,947,516

PROTECTING DOCUMENTS, NEWSPAPERS,  
AND THE LIKE

Joseph Broadman, New York, N. Y.

Application October 18, 1932. Serial No. 638,298

8 Claims. (Cl. 154—40)

My invention relates to a new and improved method of protecting documents, newspapers, and the like, and to a new and improved protected document, newspaper and the like.

One of the objects of my invention is to protect newspaper clippings and the like so that the paper will be substantially immune to the effect of age, air, moisture, handling and the like.

Another object of my invention is to protect newspapers and the like so that a clipping is strengthened and it is also provided with a protective coating which prevents deterioration by age, moisture, air, and other causes.

Another object of my invention is to provide a simple and efficient method for protecting a newspaper or the like.

Another object of my invention is to provide a method of protecting a newspaper or the like so that the printed matter on the newspaper will not be affected, and it will be possible to clearly read said printed matter.

Other objects of my invention will be set forth in the following description and drawing which illustrates a preferred embodiment thereof, it being understood that the above general statement of the objects of my invention is intended to generally explain the same, without limiting it in any manner.

For many years it has been well known that newspapers, which are ordinarily printed on wood pulp paper, rapidly deteriorate with age, especially if the newspapers are handled. For this reason it has been very difficult to preserve newspaper clippings and no practical method has hitherto been devised for efficiently and properly protecting newspaper clippings. It has been suggested to print special editions of newspapers on rag paper, in order to preserve the same, but this paper is fragile and very expensive.

According to my invention, a document, such as a newspaper or the like, is greatly strengthened without covering the newspaper in such manner as to make it difficult to read the same, and the newspaper is also sealed by means of a coating which is impermeable to air, moisture, and the like, so that the clipping can be handled and preserved indefinitely.

As shown in the annexed diagrammatical drawing, the sheet of newspaper has affixed to each face thereof a thin sheet of transparent or translucent paper.

While I do not wish to limit myself to any particular type of light-permeable paper, I prefer to use the type of paper which is referred to in the trade as "Glassine". This Glassine paper is

manufactured from sulphite pulp made from spruce wood, and the transparency is obtained by thoroughly hydrating the stock in the beaters. The glossy finish of the paper is obtained by running the paper between a series of pairs of rollers with the use of pressure and friction, similar to the ironing in a laundry.

This paper contains no wax, oil, or other coating material, as the transparency is secured without the use of any foreign material. If desired, this Glassine paper may contain sizing and an alum, and it may also contain a suitable tinting material.

The thin sheets of light-permeable paper are connected to the intermediate sheet of newspaper by means of any suitable adhesive. This adhesive is preferably a paste which is made by intermixing cold water with wheat flour. Any suitable adhesive could be employed, including adhesives which are soluble in water, and adhesives which are water-resistant. A thin film of this adhesive may be applied to the transparent paper or to the sheet of newspaper, and suitable pressure, such as rolling or rubbing pressure, is applied so as to cause the sheet of newspaper and the sheets of transparent paper to dry and adhere to each other without any wrinkles or irregularities. The three connected sheets of paper are then allowed to dry, the drying operation being conducted preferably at an ordinary room temperature of about 70° F. The sheets of transparent paper increase the strength and tearing resistance of the sheet of newspaper, so that it can be freely handled without crumpling or tearing.

However, I have discovered that the mere affixing of the sheets of transparent paper will not protect the newspaper clippings or the like from the influence of air, age, and moisture. I therefore provide a protective coating on both of the outer faces of the sheets of light-permeable paper, and this protective coating also preferably extends around the edges of the newspaper clipping or the like. This hermetically seals the paper to be protected.

It is to be understood that the invention not only applies to newspaper clippings but to the preservation of books, and other printed documents, or the like.

While I do not wish to limit myself to any specific composition for the protective coating, I prefer to use a composition which consists of a mixture of 25 parts of Manila gum or Manila copal, and 75 parts of ethyl alcohol. These proportions are by weight so that 25% by weight

of the composition consists of the Manila gum. The solution of the Manila gum in the ethyl alcohol has the consistency of a thin cream. Instead of using Manila gum, I can use a solution of East India gum in alcohol, or a solution of Pontianac gum in alcohol, said gums being dissolved in ethyl alcohol, in the proportions previously mentioned.

The coating is applied by means of a rigid pad or spreading tool or perforated roller having an outer covering of cloth or the like, so that a smooth and light-permeable coating is formed. The alcohol dries quickly.

Experience has shown that numerous coating materials penetrate the transparent paper and that such coating materials affect the ink, so that the ink is dissolved and the printed impression is blurred.

The improved coating compositions above described have sufficient body or viscosity and the alcohol evaporates with sufficient rapidity so that the protective material forms a protective coating around the clipping and the sheets of light-permeable paper. This protective coating preferably extends around the edges of the clippings and of the sheets of transparent paper so as to completely and hermetically seal the clipping. The protected clipping can be immersed in water for a long time without being affected by the moisture. If ethyl alcohol (which may be suitably denatured) is used as the solvent for the protective material, the alcohol does not pass through the transparent paper. Hence, the alcohol does not attack the printing ink. The use of alcohol is likewise advantageous because alcohol will not rapidly attack the printing ink under normal conditions. The film of gum is extremely flexible and adherent and light-permeable and it has a very slight gloss, so that said film of gum does not reflect the light too much. While the protective film of gum appears to be smooth to the naked eye, examination thereof with a magnifying glass shows that said film of gum has a slight grain or surface irregularity, which diminishes the gloss thereof. The use of the Manila gum improves the ease with which the printed matter can be read. The coating material can be applied by hand or by the use of a very simple machine and the application of said improved coating material does not require the use of heat or pressure, and the application of said coating material is not dependent upon the humidity of the atmosphere. The special Glassine light-permeable paper which I prefer to employ is slightly permeable to water or the like. Water will drip through said light-permeable paper if said paper is held in contact with the water for many hours. Hence, the water paste penetrates the light-permeable paper but only very slightly. The water paste which has been specified is preferable, because it does not exert any injurious effect upon the paper. It is only necessary to apply a single coating of the Manila gum, because the coating solution is not readily absorbed by the light-permeable paper. The light-permeable paper is not impermeable to air, but it is rendered impermeable to air by the application of the protective material.

While I have stated a preferred embodiment of my invention, I do not wish to be limited to the above mentioned details.

For example, the transparent paper could be of the type which is made by applying a solution of Canada balsam in turpentine oil to ordinary

paper. Likewise, any suitable tracing paper or tracing which has been rendered transparent by the use of oils and waxes could be utilized.

The transparent coating may be made by dissolving copal and camphor in oil of turpentine. Numerous transparent lacquers which contain various cellulose compounds, such as cellulose acetate, nitro-cellulose, celluloid, etc. may be utilized. A number of such transparent coating materials are set forth for example on page 2616 of Worden's "Technology of Cellulose Esters".

One of the essential features is to apply a thin film of coating material which is dissolved in a solvent which rapidly evaporates, so that the solvent does not pass through the transparent paper, and attack the printing ink, since the ordinary commercial solvents which are used in lacquers and varnishes attack the printing ink. Likewise, the varnish or lacquer should not contain an excess of solvent and for this purpose a minimum amount of solvent can be employed, much less in proportion than in the example which has been specifically given. Likewise, while the transparent paper should be thin, it should be thick enough to prevent the penetration of the solvent of the varnish or lacquer, through said transparent paper, under working conditions. Likewise, the solvent evaporates very rapidly so as to prevent said penetration and the paper is penetrated very slowly. Hence the solvent evaporates before it can penetrate through the transparent paper.

A ream of sheets of said transparent paper, 24" by 36", has a weight of twenty to twenty-five pounds.

Wherever I have referred to a newspaper clipping, it is to be understood that I include books and the like.

While I prefer to protect both sides of the sheet of printed paper, and to apply the protective coating to both protective sheets of transparent paper, I do not wish to be limited to this complete combination. In some cases, it may be sufficient to apply only a single sheet of transparent coated paper to the printed face of the paper which is to be protected, if only one face of the paper is written or printed upon. When I refer to a sheet of printed paper, I wish to include a sheet of paper which may have been written upon, or which may have been marked with the use of a typewriter, etc.

Likewise, I do not wish to be limited to the sequence of operations which have been mentioned herein, because the protective coating of varnish may be first applied to the transparent paper, the solvent allowed to evaporate, and the coated sheet of paper may then be connected to the sheet of paper which is to be protected. The coating can then be applied to the edges, either by applying the preparation, or spreading. In such case, it is preferable to apply the protective material to the transparent paper in the form of a coating which does not penetrate to that side of the protective paper which is to be applied to paper to be protected.

For example a film of adhesive may be applied to one side of the transparent or protective paper and the coating material may be applied to the other side thereof. This could be done in any suitable machine, and the film of adhesive could be allowed to dry. Any suitable gum adhesive could be utilized for this purpose. It would then be merely necessary for the user to moisten the film of adhesive, and connect the transparent and coated paper to the sheet of printed paper.

However, I prefer to use an adhesive of the

type specified, which can be applied to the coated transparent paper.

The transparent paper may be treated on both sides with the protective material, and it may be saturated as much as possible with said protective material. The solvent can then be allowed to evaporate, and the protective paper can then be connected to the printed paper.

I claim:

- 10 1. A method of protecting a flexible sheet of printed paper, which consists in connecting an additional flexible sheet of light-permeable material to each side of said sheet of printed paper, each said additional sheet being connected to the printed sheet by means of an intermediate layer of adhesive which is caused to enter and to penetrate only the inner part of the additional sheet, and then directly coating the exterior surface of each said additional sheet with a layer of light-permeable protective material which is caused to enter said additional sheet and to penetrate only the outer part of said sheet, said layer of protective material being flexible and non-peeling and having a resin base.
- 20 2. A method of protecting a flexible sheet of printed paper, which consists in connecting an additional flexible sheet of light-permeable material to each side of said sheet of printed paper, each said additional sheet being connected to the printed sheet by means of an intermediate layer of water-miscible adhesive which is caused to enter and to penetrate only the inner part of the additional sheet, and then directly coating the exterior surface of each said additional sheet with a layer of light-permeable protective material which is caused to enter said additional sheet and to penetrate only the outer part of said sheet, said layer of protective material being flexible and non-peeling and having a resin base.
- 30 3. A method of protecting a sheet of printed paper, which consists in connecting additional flexible sheets of light-permeable material to both sides of said sheet of printed paper by means of a water-miscible adhesive which is permitted to enter only the inner part of each sheet of light-permeable material, allowing said adhesive to dry, and then directly coating said sheets of light-permeable material with a solution of protective and light-permeable material, which is caused to penetrate said additional sheets, while causing the solvent in said solution of protective material to evaporate before it has penetrated to the ink on said printed paper, said layer of protective material being flexible and non-peeling and having a resin base.
- 40 4. A method of protecting a sheet of printed paper, which consists in connecting additional flexible sheets of light-permeable material to both sides of said sheet of printed paper by means of a water-miscible adhesive which is permitted to enter only the inner portion of each sheet of light-permeable material, allowing said adhesive

to dry, and then directly coating said sheets of light-permeable material with a protective material which consists substantially of a solution of a resin in alcohol which is caused to penetrate said additional sheets, while causing the alcohol to evaporate before it penetrates to the ink on said printed paper, said coating having a resin base.

5. A method of protecting a sheet of printed paper, which consists in connecting additional flexible sheets of light-permeable material to both sides of said sheet of printed paper by means of a water-miscible adhesive which is permitted to enter and to penetrate only the inner portion of each sheet of light-permeable material, allowing said adhesive to dry, and then directly coating said sheets of light-permeable paper with a protective material which consists substantially of a solution of Manila gum in alcohol, said solution being caused to penetrate said additional sheets.

6. A sheet of printed paper having over its printed matter to be protected, a protective sheet of light-permeable material connected to said printed paper by means of an intermediate layer of adhesive, said adhesive having entered and being confined in said light-permeable paper to that portion thereof which is adjacent the printed paper, the outer surface of the light-permeable paper having a thin and flexible and light-permeable coating of material which has penetrated the outer surface of said sheet of light-permeable paper, said protective sheet and its coating having high flexibility so that the printed paper and its protective sheet has the flexibility of a sheet of paper.

7. A sheet of printed paper having over its printed matter to be protected, a protective sheet of light-permeable material connected to said printed paper, by means of an intermediate layer of adhesive, said adhesive having entered and being confined in said light-permeable material to that portion thereof which is adjacent the printed paper, the outer surface of the light-permeable paper having a thin and flexible and light-permeable coating of material which has penetrated the outer surface of said sheet of light-permeable paper, said surface protective coating consisting substantially of a resin.

8. A sheet of printed paper having over its printed matter to be protected, a protective sheet of light-permeable material connected to said printed paper by means of an intermediate layer of adhesive, said adhesive being confined in said light-permeable material to that portion thereof which is adjacent the printed paper, the outer surface of the light-permeable paper having a thin and flexible coating of material which has penetrated the outer surface of said sheet of light-permeable material, said surface protective coating consisting substantially of Manila gum.

JOSEPH BROADMAN.